

## UNITED STATES PATENT OFFICE

2,406,453

## TREATMENT OF PAPER OR TEXTILE FABRICS

William Charlton, Stanley Graham Jarrett, and Eric Everard Walker, Blackley, Manchester, England, assignors to Imperial Chemical Industries Limited, a corporation of Great Britain

No Drawing. Application March 8, 1944, Serial No. 525,603. In Great Britain February 15, 1943

8 Claims. (Cl. 117—139.5)

1

This invention relates to a treatment of paper or textile fabrics and more particularly to new methods of finishing such materials.

In the specification of British application No. 11,780/42 there is described a method of subjecting materials consisting of or containing wool fibres at elevated temperatures to the combined action of water-vapour and the vapour of a volatile monomeric monovinylidene compound, for example, an ester of acrylic or methacrylic acid, styrene or a vinyl ester.

According to the present invention we provide a process for treating paper or textile fabrics which comprises exposing said materials to the vapour of one or more monomeric readily polymerisable compounds in the presence of persulphuric acid or a water-soluble persulphate and in the presence of a water-soluble oxy-acid of sulphur with reducing properties or a water-soluble salt of an oxy-acid of sulphur with reducing properties.

The paper may be of any kind within the common meaning of the term. The textile fabrics may be woven or knitted and composed of fibres which may be animal or vegetable, for example wool, cotton or jute; or of vegetable origin, for example viscose or acetate rayon; or entirely synthetic, for example synthetic linear polyamide (nylon) fibres; or mixtures of such fibres.

The monomeric readily polymerisable compounds are those containing the group  $\text{CH}_2=\text{C}$ : and they include, for example, acrylic acid, methacrylic acid, esters of acrylic acid, esters of methacrylic acid, acrylonitrile, vinyl esters, vinyl ethers and styrene. Of these, the lower alkyl or alkylene esters of acrylic acid and of methacrylic acid, for example, methyl and ethyl acrylates and methacrylates, are especially suitable; the higher alkyl esters (wherein the alkyl group has more than 6 carbon atoms), for example, 2-ethylhexyl methacrylate and octadecyl methacrylate, are less suitable since they polymerise more slowly or to a lesser extent under the conditions employed.  $\beta$ -Ethoxyethyl methacrylate and  $n$ -butyl methacrylate are also very suitable, the former being the more easily polymerised, due probably to its greater solubility in water caused by the presence of the ether grouping. Unsaturated esters such as diallyl maleate are also suitable. Vinyl esters, particularly the inorganic esters, are less suitable since they polymerise very slowly under the conditions employed. In general, the monomeric readily polymerisable compounds used should have high vapour pressures at temperatures below 100° C., so as to obviate the need for using tem-

2

peratures substantially higher than 100° C. for vapourising substantial proportions of said compounds; heating at temperatures above 100° C. is not desirable, since such heating tends to dry off the fabric and to destroy the efficacy of polymerisation catalyst and activator.

The exposure of the paper or fabric to the monomeric polymerisable compounds under the conditions herein described, causes these compounds to be polymerised on the paper or fabric in a much shorter time than has hitherto been found possible. Frequently, it has been found that deposition of the polymers can be effected rapidly at temperatures as low as 30° C. or even lower, although, with some monomers, working at higher temperatures, for example, 60–70° C., is preferred.

The persulphuric acid or the persulphate, for example ammonium persulphate, is conveniently applied to the paper or fabric, before exposure to the vapours of the monomer, by soaking said materials in or impregnating with a dilute aqueous solution thereof. Usually, the water is not removed from the paper or fabric prior to the exposure to the vapours of the monomeric readily polymerisable compound, since it is preferable for the paper or fabric to be moist with water; if the paper or fabric is dry, polymerisation is extremely slow. A 2% solution of ammonium persulphate, used so that the amounts of solution retained by the fabric or paper are from one to two times the weight of the fabric or paper, has been found to give satisfactory results. Weaker solutions, for example 0.5%, may be used if desired.

The exposure to the vapour of the monomers is conveniently carried out by entraining the vapour in an oxygen-free gas, such as carbon dioxide or nitrogen and then interposing the paper or fabric in a stream of the gas and vapour. Inert volatile liquids such as water or an alcohol may be mixed with the compound being vapourised. The exposure may be at atmospheric or elevated temperatures.

Examples of suitable water-soluble salts of oxy-acids of sulphur with reducing properties are sulphites, hydrosulphites, sulphonylates, pyrosulphites, bisulphites, and thiosulphates, in particular the sodium salts. These are conveniently applied to the paper or fabric, as by soaking in or impregnating with dilute aqueous solution thereof, and they are usually used in amounts less than the amounts of the persulphuric acid or water-soluble persulphate used. Alternatively, when using a free acid, for instance sulphurous acid, sulphur dioxide in admixture with water

vapour may be entrained with the vapour of the monomer in a carrier gas. Or, gaseous sulphur dioxide in admixture with a carrier gas may be passed through the paper or fabric which is moist with water.

The effects produced vary with the nature of the paper or the fabric, the monomer and the amount of polymer deposited, and may be modified by using more than one monomer. When using more than one monomer, it is sometimes advantageous to use a mixture comprising both slow and rapid polymerising monomers. It is often advantageous to repeat the treatment, in accordance with the invention once or more than once, since by so doing unexpectedly large quantities of polymers are formed on the paper or fabric. The deposition of small amounts of the polymers on the paper or fabrics causes small changes in handle. The amounts of polymer deposited depend on the conditions of working, and may be varied as desired in accordance with experience gained by trial.

The invention is illustrated but not limited by the following examples, in which, unless otherwise stated, the parts are expressed by weight:

*Example 1*

Cotton fabric is impregnated with a cold solution of ammonium persulphate (1 part) and sodium hydrosulphite (0.5 part) in water (98.5 parts), and excess of the solution removed by squeezing or passing between rollers. The fabric is suspended in the upper part of a cylindrical vessel in the bottom of which is placed methyl acrylate in excess of the amount to be polymerised on the fabric. Carbon dioxide is bubbled through the methyl acrylate, and the vessel is heated in a water bath at 40-60° C. for as long as required. Depending on the rate of flow of carbon dioxide, the temperature of the vessel, the relative weights of monomer and fabric, and the time varying amounts of monomer are deposited and polymerised on the fabric. For instance a gain in weight of 80% of the fabric weight is obtained in about 30 minutes. When sufficient polymer is formed on the fabric, it is rinsed in warm water and dried.

Depending on the amount of polymer formed on the fabric, different effects are produced. Thus the deposition of a small amount of polymer gives a soft handle, whereas a large amount gives a fabric resembling oiled-silk in appearance.

*Example 2*

A stream of carbon dioxide is bubbled successively through a saturated solution of sulphur dioxide in water at 20° C., then through methyl methacrylate at 25° C., a sintered glass distributor being used to give a good contact between gas and monomer. The carbon dioxide, which carries entrained with it small amounts of methyl methacrylate and sulphur dioxide is passed upwards through a shallow horizontal chamber kept at 20-25° C. Cotton fabric which has previously been impregnated with a dilute solution of 2 parts of ammonium persulphate in 98 parts of water and squeezed to remove excess of the solution, is placed in the chamber so that the gas stream passes through the fabric. Methyl methacrylate polymer forms rapidly on the fabric, for instance, to the extent of 50% of the weight of the fabric in 30 minutes. When sufficient polymer is formed on the fabric, it is removed, washed with water, and dried.

Under similar conditions, but with the monomer maintained at 90° C., so that the fabric in the

chamber is at about 60° C., vinyl acetate polymer is formed to the extent of about 7% of the fabric weight during 2 hours.

Under similar conditions, but with the monomer maintained at 100° C., diallyl maleate polymer is formed to the extent of about 43% of the fabric weight during 2 hours.

*Example 3*

10 Methyl methacrylate is caused to polymerise in the manner described in Example 2 on fabrics composed of viscose rayon and of polyhexamethylene adipamide (nylon) yarn, respectively. Polymerisation is continued until an increase in weight of 18% is obtained in the case of the viscose rayon fabric and until an increase in weight of 25-30% is obtained in the case of the polyhexamethylene adipamide fabric. In both cases the fabrics are delustered by the treatment.

20

*Example 4*

Acrylonitrile is caused to polymerise on a variety of fabrics in the manner described in Example 2. At temperatures of 20-25° C., the following amounts of acrylonitrile polymer are deposited in the times stated:

On cotton fabric----- 55% by weight of the cloth in 45 minutes.  
On viscose rayon fabric--- 25% by weight of the cloth in 45 minutes.  
30 On woollen fabric----- 10% by weight of the cloth in 35 minutes.

The cotton fabric is stiffened, the viscose rayon fabric is stiffened and delustered by the treatment, and the woollen fabric has a fuller handle. The effects are not destroyed by boiling the fabrics in aqueous 5% soap and the 1% soda solutions, but a yellow colour develops.

40

*Example 5*

A stream of carbon dioxide is bubbled through a saturated solution of sulphur dioxide in water at 20° C., then through methyl acrylate at 25° C. The carbon dioxide, which carries entrained with it small amounts of methyl acrylate and sulphur dioxide is passed upwards through a shallow, unheated, horizontal chamber. Cotton fabric which has previously been impregnated with a dilute solution of 2 parts of ammonium persulphate in 98 parts of water and squeezed to remove excess of the solution, is placed in the chamber so that the gas stream passes through it. The rate of passage of the carbon dioxide is 4.3 gms./sq. cm. of fabric/hr. After 30 minutes treatment methyl acrylate polymer is formed on the fabric to the extent of 93% of the fabric weight.

If the flow of carbon dioxide is increased to 8.6 gms./sq. cm. of fabric/hr. the amount of polymer formed in the same time falls to 74% of the fabric weight.

*Example 6*

The recipe of Example 5 is employed to form  $\beta$ -ethoxyethyl methacrylate polymer on a cotton fabric. At a rate of flow of carbon dioxide of 2.15 gms./sq. cm. of fabric/hr., the amount of polymer formed on the fabric in 30 minutes is 10.5% of the fabric weight. When the temperature of the  $\beta$ -ethoxyethyl methacrylate is increased to 50° C. or 75° C. the amounts of polymer deposited in the same time are 23% and 46.5% of the fabric weight, respectively.

Under similar conditions, using a mixture of equal parts of ethyl alcohol and 2-ethylhexyl methacrylate, the temperature of this mixture

75

being 50° C., the amount of polymer deposited in the same time is 6% of the fabric weight.

Under similar conditions, using a mixture of equal parts of methyl methacrylate and 2-ethylhexyl methacrylate, the temperature of this mixture being 50° C., the amount of polymer deposited in the same time is 42% of the fabric weight.

*Example 7*

The recipe of Example 5 is used to form *n*-butyl methacrylate polymer on a cotton fabric, the temperature of the monomer being 50° C. The amount of polymer formed on the fabric in 30 minutes is 4% of the fabric weight, when the rate of flow of carbon dioxide is 4.3 gms./sq. cm. of fabric/hr.

When the treatment is repeated, including the step of impregnating the fabric with the solution of ammonium persulphate, the total amount of polymer deposited is 54% of the weight of fabric, and, by a third treatment, this is increased to 150%. If the step of impregnating with ammonium persulphate solution is omitted in the second and third treatments, then the total amount of polymer deposited in three treatments is only 6%.

*Example 8*

The recipe of Example 5 is used to form methacrylic acid polymer on a woollen fabric. The amount of polymer formed on the fabric in 30 minutes is 32% of the fabric weight, when the rate of flow of carbon dioxide is 4.3 gms./sq. cm. of fabric/hr.

When the temperature of the methacrylic acid is increased from 25° C. to 40° C., the amount of polymer formed on the fabric in the same time is 45% of the fabric weight.

*Example 9*

The recipe of Example 5 is used to form styrene polymer on absorbent paper, the temperature of the monomer being 50° C., and the rate of flow of carbon dioxide being 4.3 gms./sq. cm. of fabric/hr. After treatment for 30 minutes, the paper gains in weight by only 2%, but after impregnating the paper again with the persulphate solution and treating for a further 30 minutes, the total gain in weight is 24.5%. After a third treatment, the amount of polymer deposited corresponds to a total increase in weight of 119%.

*Example 10*

The recipe of Example 5 is used to polymerise on a cotton fabric a mixture of equal parts of acrylonitrile and vinyl isobutyl ether, the temperature of the mixture of monomers being 50° C., and the rate of flow of carbon dioxide being 4.3 gms./sq. cm. of fabric/hr. The amount of polymeric material formed on the fabric in 30 minutes is 10% of the fabric weight.

10 We claim:

1. A process for treating fibrous material which comprises applying to said material an aqueous solution of a member of the class consisting of persulfuric acid and water soluble persulfates, exposing said material while moist with water to the vapor of a readily polymerizable compound containing the group  $\text{CH}_2=\text{C}$ : in the further presence of a member of the class consisting of water soluble oxy-acids of sulfur with reducing properties and water soluble salts of oxy-acids of sulfur with reducing properties and simultaneously polymerizing said polymerizable compound on said material during the exposure of said material to said vapor.
2. The process of claim 1 wherein the monomeric, readily polymerizable compound is an ester of an acrylic acid, the hydrocarbon group component of the ester containing not in excess of six carbon atoms.
3. The process of claim 1 wherein the monomeric, readily polymerizable compound has a high vapor pressure at temperatures below 100° C.
4. The process of claim 1 wherein the persulfuric compound is ammonium persulfate.
5. The process of claim 1 wherein the sulfur compound is a sodium salt.
6. The process of claim 1 wherein the sulfur compound is sulfurous acid.
7. The process of claim 1 wherein the sulfur compound is introduced in admixture with water vapor by entrainment with the vapor of the monomer in a carrier gas.
8. The process of claim 1 wherein the sulfur compound is formed by introducing sulfur dioxide in admixture with a carrier gas.

WILLIAM CHARLTON.

STANLEY GRAHAM JARRETT.

ERIC EVERARD WALKER.